



resistance section is smaller than a thickness reduction rate of the high deformation resistance section.

**16 Claims, 10 Drawing Sheets**

**(58) Field of Classification Search**

CPC ..... B21D 41/028; B21D 41/04; B21D 39/08;  
B21D 51/00; B21D 51/16; B21D 19/08;  
B21D 19/082; B21D 3/00; B21D 3/005;  
B21D 39/203

See application file for complete search history.

(56)

**References Cited**

U.S. PATENT DOCUMENTS

|              |      |        |       |       |            |           |
|--------------|------|--------|-------|-------|------------|-----------|
| 7,225,868    | B2 * | 6/2007 | Arai  | ..... | B21C 1/24  |           |
|              |      |        |       |       |            | 166/277   |
| 2009/0139295 | A1 * | 6/2009 | Motoo | ..... | B21D 39/20 |           |
|              |      |        |       |       |            | 72/370.06 |

FOREIGN PATENT DOCUMENTS

|    |             |            |                  |
|----|-------------|------------|------------------|
| JP | 2002-346664 | 12/2002    |                  |
| JP | 2003-126930 | A 5/2003   |                  |
| JP | 2006-272350 | * 10/2006  | ..... B21D 41/02 |
| JP | 2006-272350 | A 10/2006  |                  |
| JP | 2009-50888  | A 3/2009   |                  |
| JP | 2009-136897 | A 6/2009   |                  |
| JP | 4798875     | B2 10/2011 |                  |
| JP | 5221910     | B2 6/2013  |                  |

OTHER PUBLICATIONS

Written Opinion of the International Searching Authority for PCT/JP2015/086239 (PCT/ISA/237) dated Feb. 9, 2016.

Chinese Office Action dated May 3, 2018, issued in Chinese Counterpart application No. 201580070248.8.

\* cited by examiner

FIG. 1A



FIG. 1B



FIG. 1C



FIG. 2



FIG. 3



FIG. 4A



FIG. 4B



FIG. 5A



FIG. 5B



FIG. 6A



FIG. 6B



FIG. 7A



FIG. 7B



FIG. 8A



FIG. 8B



FIG. 8C



FIG. 9



FIG. 10A



FIG. 10B



FIG. 11



FIG. 12



## METHOD OF MANUFACTURING FLARING-PROCESSED METAL PIPE

### TECHNICAL FIELD OF THE INVENTION

The present invention relates to a method of manufacturing a flaring-processed metal pipe.

Priority is claimed on Japanese Patent Application No. 2014-264337, filed on Dec. 26, 2014, the content of which is incorporated herein by reference.

### RELATED ART

As a method of manufacturing a flaring-processed metal pipe, a method of press-fitting a tapered pipe expansion punch (punch) from an open end of a metal pipe (raw pipe) which is a material and expanding the metal pipe in the radial direction thereof to form a pipe expanded section in the metal pipe is known (for example, refer to Patent Documents 1 and 2).

However, in the above-described manufacturing method, due to various factors, forming defects such as cracks in the pipe expanded section or buckling at the root of the pipe expanded section occur. Accordingly, it is required to prevent the occurrence of the above-described forming defects when the flaring-processed metal pipe is manufactured (the metal pipe is expanded and formed) from a raw pipe.

### PRIOR ART DOCUMENT

#### Patent Documents

[Patent Document 1] Japanese Patent No. 4798875  
[Patent Document 2] Japanese Patent No. 5221910

### DISCLOSURE OF THE INVENTION

#### Problems to be Solved by the Invention

The inventors focused on a thickness distribution and a hardness distribution in the circumferential direction of the raw pipe as a cause of forming defects in the pipe expansion forming (pipe expansion processing) of the metal pipe.

FIG. 10A is a cross-sectional view showing an example of a thickness distribution of an electric resistance welded steel pipe 301 used as a material for pipe expansion forming, and FIG. 10B is a cross-sectional view showing an example of a thickness distribution of a seamless steel pipe 302 used as a material for the pipe expansion forming. In addition, FIG. 11 is a graph showing the thickness distribution of the electric resistance welded steel pipe 301 in the circumferential direction. In FIG. 11, a horizontal axis indicates an angle from a seam, that is, an angle from a weld 305 formed on the electric resistance welded steel pipe 301.

As shown in FIGS. 10A and 11, in the electric resistance welded steel pipe 301, a thickness  $t_1$  of a portion where the angle from the weld 305 is approximately  $60^\circ$  and a thickness  $t_2$  of a portion where the angle is approximately  $150^\circ$  are smaller than the thicknesses  $t_3$  to  $t_5$  of the other portions, and a thickness deviation occurs. Moreover, the thicknesses  $t_1$  and  $t_2$  are approximately 98% to 99% of the average value of the thicknesses.

In addition, as shown in FIG. 10B, in the seamless steel pipe 302, a thickness deviation occurs in which the thickness  $t_7$  is smaller than the thickness  $t_8$  and the thickness  $t_9$  is satisfied.

FIG. 12 is a graph showing the hardness distribution (strength distribution) of the electric resistance welded steel

pipe 301 in the circumferential direction. Moreover, in FIG. 12, a horizontal axis indicates the position in the circumferential direction with the position of the weld of the electric resistance welded steel pipe 301 as a reference. As shown in FIG. 12, in the electric resistance welded steel pipe 301, a HAZ softened region exists near the weld. This HAZ softened region has a relatively lower hardness than those of other regions and has a hardness of approximately 90% of the average hardness.

As described above, the electric resistance welded steel pipe 301 has a non-uniform thickness distribution and hardness distribution in the circumferential direction, and the seamless steel pipe 302 has a non-uniform thickness distribution in the circumferential direction. When the electric resistance welded steel pipe 301 (or the seamless steel pipe 302) having the non-uniform distribution is uniformly flared and formed (expanded and formed) in the circumferential direction, a force which expands the electric resistance welded steel pipe 301 (or the seamless steel pipe 302) uniformly acts in the circumferential direction. In addition, since a deformation resistance is small in a section having a thin thickness (thin section) and a section having a low hardness (low hardness section), the deformation concentrates in these sections. As a result, despite the fact that a pipe expansion rate is much lower than deforming capacity of the steel pipe, forming defects such as breakage easily occur since thickness reduction rates of these sections are larger than the thickness reduction rates of the other sections.

The present invention is made in consideration of the above-described circumstances, and an object thereof is to provide a method of manufacturing a flaring-processed metal pipe in which it is possible to prevent occurrence of forming defects such as breakage when the flaring-processed metal pipe is manufactured from a hollow shell including a portion having a relatively small deformation resistance.

#### Means for Solving the Problem

In order to solve the above problem, the present invention adopts the following.

(1) According to an aspect of the present invention, there is provided a method of manufacturing a flaring-processed metal pipe having a pipe expanded section from a hollow shell including a plurality of portions having different deformation resistances when viewed in a circumferential direction, the method including: among the plurality of portions, specifying a portion having a relatively small deformation resistance as a low deformation resistance section, and a portion having a relatively larger deformation resistance than that of the low deformation resistance section as a high deformation resistance section; and press-fitting a pipe expansion punch into the hollow shell and expanding the hollow shell, in the press-fitting and the expanding, a thickness reduction rate of the low deformation resistance section is smaller than a thickness reduction rate of the high deformation resistance section.

(2) In the aspect described in the above (1), it may be configured as follows: the pipe expansion punch includes a first abutment surface which abuts the low deformation resistance section of the hollow shell, and a second abutment surface which abuts the high deformation resistance section of the hollow shell, and an inclination angle of the first abutment surface with respect to the central axis of the pipe expansion punch is smaller than an inclination angle of the second abutment surface with respect to the central axis, and in the press-fitting and the expanding, the pipe expansion

punch is press-fitted into the hollow shell while the first abutment surface of the pipe expansion punch abuts the low deformation resistance section of the hollow shell and the second abutment surface of the pipe expansion punch abuts the high deformation resistance section of the hollow shell.

(3) In the aspect described in the above (2), the inclination angle of the first abutment surface of the pipe expansion punch may be  $0^\circ$ .

(4) In the aspect described in the above (2) or (3), it may be configured as follows: the press-fitting and the expanding include press-fitting the pipe expansion punch into the hollow shell to obtain an intermediate formed product from the hollow shell, and press-fitting a forming punch having a shape which coincides with an inner surface of the pipe expanded section of the flaring-processed metal pipe into the intermediate formed product.

(5) In the aspect described in the above (4), in the press-fitting of the pipe expansion punch, the pipe expansion punch may be press-fitted into the hollow shell such that a diameter expansion amount of the low deformation resistance section of the hollow shell is less than 0.5 times a diameter expansion amount of the high deformation resistance section of the hollow shell.

(6) In the aspect of any one of the above (1) to (5), the hollow shell may be an electric resistance welded steel pipe or a seamless steel pipe.

#### Effects of the Invention

According to each of the aspects of the present invention, it is possible to prevent occurrence of forming defects such as breakage when a flaring-processed metal pipe is manufactured from a hollow shell including a portion having a relatively small deformation resistance.

#### BRIEF DESCRIPTION OF THE DRAWINGS

FIG. 1A is a front view showing a hollow shell and a pipe expansion punch used in a method of manufacturing a flaring-processed metal pipe according to a first embodiment of the present invention.

FIG. 1B is a sectional view taken along line A-A of the hollow shell and the pipe expansion punch shown in FIG. 1A.

FIG. 1C is a schematic perspective view showing the pipe expansion punch.

FIG. 2 is a sectional view showing a state in which the pipe expansion punch is press-fitted into the hollow shell.

FIG. 3 is a sectional view showing a state in which a forming punch is press-fitted to an intermediate formed product obtained by expanding the hollow shell using the pipe expansion punch.

FIG. 4A is a sectional view showing a first modification example of the method of manufacturing the flaring-processed metal pipe.

FIG. 4B is a sectional view showing the continuation of the manufacturing method according to the modification example.

FIG. 5A is a sectional view showing a second modification of the method of manufacturing the flaring-processed metal pipe.

FIG. 5B is a sectional view showing the continuation of the manufacturing method according to the modification example.

FIG. 6A is a view showing a third modification example of the method of manufacturing the flaring-processed metal

pipe, and is a front view showing a pipe expansion punch and a hollow shell used in the modification example.

FIG. 6B is a schematic perspective view showing the pipe expansion punch.

FIG. 7A is a view showing a fourth modification example of the method for manufacturing the flaring-processed metal pipe, and is a front view showing a pipe expansion punch and a hollow shell used in the modification example.

FIG. 7B is a schematic perspective view showing the pipe expansion punch.

FIG. 8A is a sectional view showing a hollow shell and a pipe expansion punch used in a method of manufacturing a flaring-processed metal pipe according to a second embodiment of the present invention.

FIG. 8B is a view for explaining the method of manufacturing the flaring-processed metal pipe, and is a sectional view showing a state in which the pipe expansion punch is press-fitted into the hollow shell.

FIG. 8C is a sectional view showing the continuation of the method of manufacturing the flaring-processed metal pipe.

FIG. 9 is a diagram showing a hardness distribution of a hollow shell used in Example 2.

FIG. 10A is a cross-sectional view showing an electric resistance welded steel pipe and is a view showing an example of a thickness distribution of the electric resistance welded steel pipe.

FIG. 10B is a cross-sectional view showing a seamless steel pipe, and a view showing an example of a thickness distribution of the seamless steel pipe.

FIG. 11 is a graph showing a thickness distribution of the electric resistance welded steel pipe in a circumferential direction.

FIG. 12 is a graph showing the hardness distribution of the electric resistance welded steel pipe in the circumferential direction.

#### EMBODIMENT OF THE INVENTION

40 Hereinafter, embodiments of the present invention will be described in detail with reference to the drawings. In the present specification and the drawings, the same reference numerals are assigned to constituent elements having substantially the same functional configuration, and overlapping description thereof will be omitted.

#### First Embodiment

50 In a method of manufacturing a flaring-processed metal pipe according to the first embodiment of the present invention, a hollow shell 1 having a hollow circular cross section shown in FIGS. 1A and 1B is expanded and formed to manufacture a flaring-processed metal pipe 20 shown in FIG. 3. The flaring-processed metal pipe 20 is composed of 55 a straight pipe section 21, a pipe expanded section 23 which is formed by expanding the end portion of the hollow shell 1, and a transition section 22 which is provided between the straight pipe section 21 and the pipe expanded section 23. In addition, for example, the flaring-processed metal pipe 20 is 60 suitably used for automotive parts and the like.

For example, the material of the hollow shell 1 used for manufacturing the flaring-processed metal pipe 20 is a metal such as iron, aluminum, stainless steel, copper, titanium, magnesium, or steel. Preferably, a value  $n$  indicating a work hardening coefficient (distortion-effect index) of the hollow shell 1 is 0.01 to 0.3 from the viewpoint of preventing occurrence of buckling, and a pressing force required for

pipe expansion forming from being excessive. Preferably, an  $r$  value indicating the deep drawability of the hollow shell 1 is 0.5 to 3 from the viewpoint of preventing occurrence of wrinkle, and the pressing force required for the pipe expansion forming from being excessive.

For example, the hollow shell 1 is an electric resistance welded pipe, a seamless pipe, a pipe manufactured by extrusion, a pipe manufactured by drawing, or the like.

FIGS. 1A and 1B are views showing the hollow shell 1 and a pipe expansion punch 50 used for expanding the hollow shell 1. In addition, FIG. 1A is a front view of the hollow shell 1 and the pipe expansion punch 50, and FIG. 1B is a sectional view taken along line A-A in FIG. 1A.

As shown in FIGS. 1A and 1B, the hollow shell 1 has a thickness  $t_1$  and a thickness  $t_2$  which is larger than the thickness  $t_1$  when viewed along the circumferential direction thereof. That is, the hollow shell 1 has a thin section 1a (low deformation resistance section) having the thickness  $t_1$  and a thick section 1b (high deformation resistance section) having a thickness  $t_2$ .

For example, the thickness  $t_1$  of the thin section 1a is less than 99% of an average thickness of the hollow shell 1. Moreover, since the thin section 1a is thinner than the thick section 1b, the thin section 1a is more likely to be deformed than the thick section 1b when pipe expansion forming is performed. In other words, the thin section 1a has less deformation resistance against a force of expanding in the radial direction than the thick section 1b.

For example, the average thickness of the hollow shell 1 is 0.5 to 30 mm, and for example, the outer diameter of the hollow shell 1 is 15 to 700 mm. Preferably, the ratio of the average thickness of the hollow shell 1 to the outer diameter of the hollow shell 1 is 0.005 to 0.3. In this case, it is possible to efficiently manufacture the flaring-processed metal pipe 20 from the hollow shell 1.

For example, the thickness of the hollow shell 1 can be obtained using a measuring instrument such as a caliper. In addition, it is possible to specify the thin section 1a and the thick section 1b by ascertaining the thickness distribution of the hollow shell 1.

As shown in FIGS. 1A to 1C, the pipe expansion punch 50 includes a cylindrical section 51 having a diameter which is larger than the outer diameter of the hollow shell 1, and a tapered section 52 which is tapered from the cylindrical section 51 toward a tip end surface 50a. The tapered section 52 is decentered with a predetermined eccentric amount with respect to the cylindrical section 51. That is, a central axis CL2 of the cylindrical section 51, and a central axis CL3 of the tapered section 52 are parallel to and separated from each other.

In addition, the tapered section 52 has a first tapered surface 52a (first abutment surface) which abuts the thin section 1a of the hollow shell 1, and a second tapered surface 52b (second abutment surface) which abuts the thick section 1b of the hollow shell 1.

The first tapered surface 52a has a taper angle  $\alpha$  (inclination angle). The second tapered surface 52b has a taper angle larger than the taper angle  $\alpha$ , and the maximum taper angle is  $\beta$ . That is, the taper angle  $\alpha$  is smaller than the taper angle  $\beta$ . Moreover, the taper angle indicates the inclination angle of the tapered surface with respect to the central axes CL2 and CL3 in a case where the pipe expansion punch 50 is viewed in a cross section including the central axes CL2 and CL3.

First, as shown in FIGS. 1A and 1B, when the flaring-processed metal pipe 20 is manufactured from the hollow shell 1, the pipe expansion punch 50 moves along the central

axis CL1 of the hollow shell 1 and is inserted into the hollow shell 1 through the opening end 2 of the hollow shell 1. At this time, the pipe expansion punch 50 is inserted into the hollow shell 1 such that the first tapered surface 52a abuts the thin section 1a of the hollow shell 1 and the second tapered surface 52b abuts the thick section 1b of the hollow shell 1.

In addition, as shown in FIG. 2, the pipe expansion punch 50 is pushed into a predetermined position in the hollow shell 1. At this time, since the pipe expansion punch 50 moves inside the hollow shell 1 while the tapered section 52 of the pipe expansion punch 50 abutting the hollow shell 1, the hollow shell 1 is spread in the radial direction thereof and is expanded along the shape of the pipe expansion punch 50. As a result, an intermediate formed product 10 shown in FIG. 2 can be obtained from the hollow shell 1.

For example, the pipe expansion punch 50 can be pushed into the hollow shell 1 using a pressurization mechanism such as a hydraulic cylinder, a gas cylinder, a spring, or a rubber.

In the above-described process, the hollow shell 1 is expanded in the radial direction while the first tapered surface 52a of the pipe expansion punch 50 abuts the thin section 1a of the hollow shell 1 and the second tapered surface 52b of the pipe expansion punch 50 abuts the thick section 1b of the hollow shell 1. At this time, since the taper angle of the second tapered surface 52b is larger than the taper angle of the first tapered surface 52a, the thick section 1b is preferentially subjected to tensile processing with respect to the thin section 1a. As a result, a thickness reduction rate of the thin section 1a of the hollow shell 1 can be smaller than the thickness reduction rate of the thick section 1b of the hollow shell 1. That is, when the hollow shell 1 is expanded, since it is possible to prevent concentration of deformation in the thin section 1a, it is possible to prevent occurrence of forming defects such as breakage in the thin section 1a.

As shown in FIG. 2, the intermediate formed product 10 includes a straight pipe section 11 which is a non-processed portion, a pipe expanded section 13, and a transition section 12 which is provided between the straight pipe section 11 and the pipe expanded section 13.

The pipe expanded section 13 of the intermediate formed product 10 has a portion 13a corresponding to the thin section 1a of the hollow shell 1 and a portion 13b corresponding to the thick section 1b of the hollow shell 1. In addition, the straight pipe section 11 of the intermediate formed product 10 has a portion 11a corresponding to the thin section 1a of the hollow shell 1 and a portion 11b corresponding to the thick section 1b of the hollow shell 1.

As described above, in the above-described process, the hollow shell 1 is expanded and formed such that the thickness reduction rate of the thin section 1a of the hollow shell 1 is smaller than the thickness reduction rate of the thick section 1b of the hollow shell 1. Therefore, in the intermediate formed product 10, a value (the thickness reduction rate of the thin section 1a) obtained by dividing a difference value (the thickness reduction amount of the thin section 1a of the hollow shell 1) between the thickness  $t_1$  of the portion 11a and a thickness  $t_1'$  of the portion 13a by the thickness  $t_1$  is smaller than a value (the thickness reduction rate of the thick section 1b) obtained by dividing a difference value (the thickness reduction amount of the thick section 1b of the hollow shell 1) between the thickness  $t_2$  of the portion 11b and a thickness  $t_2'$  of the portion 13b by the thickness  $t_2$ .

Moreover, from the viewpoint of decreasing the amount of deformation of the thin section 1a and avoiding breakage

of the thin section **1a**, the diameter expansion amount **L1** of the thin section **1a** of the hollow shell **1** is less than 0.5 times a diameter expansion amount **L2** of the thick section **1b** of the hollow shell **1**.

Here, the “diameter expansion amount” means the length of the hollow shell **1** expanded in the radial direction, and specifically, means the dimension (distance) between the inner surface of the pipe expanded section after processing and the inner surface of the hollow shell **1**. That is, as shown in FIG. 2, “the diameter expansion amount **L1** of the thin section **1a** of the hollow shell **1**” indicates the dimension between the inner surface of the portion **11a** of the intermediate formed product **10** and the inner surface of the portion **13a** of the intermediate formed product **10**. Moreover, the “diameter expanded amount **L2** of the thick section **1b** of the hollow shell **1**” indicates the dimension between the inner surface of the portion **11b** of the intermediate formed product **10** and the inner surface of the portion **13b** of the intermediate formed product **10**.

Subsequently, the intermediate formed product **10** may be formed into the flaring-processed metal pipe **20** using a forming punch **60** and a stationary die **70** shown in FIG. 3. As shown in FIG. 3, the forming punch **60** has a cylindrical section **61**, and a tapered section **62** which is tapered from the cylindrical section **61** toward the tip end surface **60a**. Unlike the pipe expansion punch **50**, in the forming punch **60**, a central axis **CL4** of the cylindrical section **61** coincides with the central axis of the tapered section **62**. That is, the cylindrical section **61** and the tapered section **62** are coaxially formed.

The cylindrical section **61** has an outer surface shape which coincides with the shape of the inner surface of the pipe expanded section **23** of the flaring-processed metal pipe **20**. The tapered section **62** has an outer surface shape which coincides with the inner surface of the transition section **23** of the flaring-processed metal pipe **20**, and has a taper angle  $\gamma$ .

As shown in FIG. 3, the stationary die **70** includes a bottom wall section **71** which abuts the end surface of the straight pipe section **11** of the intermediate formed product **10**, and a side wall section **72** which abuts the outer surface of the straight pipe section **11** of the intermediate formed product **10**. Moreover, the inner surface shape of the side wall section **72** coincides with the outer surface shape of the flaring-processed metal pipe **20**.

When the intermediate formed product **10** is formed into the flaring-processed metal pipe **20**, first, the intermediate formed product **10** is set in the stationary die **70** along the bottom wall section **71** and the side wall section **72** of the stationary die **70**. Thereafter, the forming punch **60** is pushed into the intermediate formed product **10**. As described above, since the forming punch **60** has the shape conforming to the shape of the inner surface of the flaring-processed metal pipe **20** and the side wall section **72** of the stationary die **70** has the shape conforming to the outer surface shape of the flaring-processed metal pipe **20**, it is possible to obtain the flaring-processed metal pipe **20** by pushing the forming punch **60** into the intermediate formed product **10**.

According to the method of manufacturing the flaring-processed metal pipe **20** according to the above-described present embodiment, since the hollow shell **1** is expanded using the pipe expansion punch **50**, the force for expanding the thin section **1a** of the hollow shell **1** in the radial direction is weakened while the force for expanding the thick section **1b** of the hollow shell **1** in the radial direction becomes stronger. That is, since the hollow shell **1** is expanded such that the thickness reduction rate of the thin

section **1a** of the hollow shell **1** is smaller than the thickness reduction rate of the thick section **1b** of the hollow shell **1**, it is possible to prevent concentration of deformation in the thin section **1a**, and it is possible to prevent breakage or the like of the hollow material **1**. As a result, it is possible to manufacture a flaring-processed metal pipe having a larger pipe expansion rate than that of the related art.

Moreover, according to the method of manufacturing the flaring-processed metal pipe **20** according to the present embodiment, since the hollow shell **1** is expanded such that the thickness reduction rate of the thin section **1a** of the hollow shell **1** is smaller than the thickness reduction rate of the thick section **1b** of the hollow shell **1**, it is possible to manufacture a flaring-processed metal pipe including a pipe expanded section having a uniform thickness from the hollow shell **1** having a non-uniform thickness distribution.

Here, the above-described “pipe expansion rate” means a rate at which the outer diameter of the pipe expanded section after the pipe expansion forming is performed is increased with respect to the outer diameter of the hollow shell **1**. That is, in a case where the pipe expansion rate is defined as **P** (%), the outer diameter of the pipe expanded section after pipe expansion forming performed is defined as **d1** (mm), and the outer diameter of the hollow shell **1** is defined as **d2** (mm), the pipe expansion rate **P** is represented by the following Expression (1).

$$P = ((d1 - d2) / d2) \times 100$$

Expression (1)

In addition, when the hollow shell **1** is formed into the intermediate formed product **10**, if the pipe expansion rate of the intermediate formed product **10** is decreased, effects for preventing the breakage of the thin section **1a** of the hollow shell **1** decrease. Therefore, preferably, the hollow shell **1** is formed into the intermediate formed product **10** so that the pipe expansion rate of the intermediate formed product **10** becomes 50% or more with respect to the pipe expansion rate of the flaring-processed metal pipe **20**.

In addition, compared to a case where the material of the hollow shell **1** is an aluminum alloy, in a case where the material of the hollow shell **1** is stainless steel, forming defects easily occur when the pipe expansion forming is performed. Accordingly, compared to the case where the material of the hollow shell **1** is the aluminum alloy, in the case where the material of the hollow shell **1** is stainless steel, the effects for preventing breakage in the thin section **1a** increase.

#### [Modification Example of First Embodiment]

In the present embodiment, the case where the hollow shell **1** has the thin section **1a** and the thick section **1b** (that is, the case where the thickness distribution in the circumferential direction is non-uniform) is described. However, for example, the flaring-processed metal pipe may be manufactured from a hollow shell having a non-uniform hardness distribution in the circumferential direction. In this case, the hardness distribution is ascertained by a tensile test, hardness measurement or the like, the first tapered surface **52a** of the pipe expansion punch **50** may abut a low hardness section (low deformation resistance section) having a relatively low hardness, and the second tapered surface **52b** of the pipe expansion punch **50** may abut a high hardness section (high deformation resistance section) having a relatively high hardness. In this case, for example, a portion having a hardness which is less than 95% with respect to the average value of the hardness of the hollow shell can be specified as the low hardness section.

In addition, for example, in a case where the hollow shell has both a non-uniform thickness distribution and a non-

uniform hardness distribution, a portion in which the product value between the thickness and the hardness is less than 95% of the average value is specified as the low deformation resistance section, and the first tapered surface **52a** of the pipe expansion punch **50** may abut the low deformation resistance section.

In addition, in the present embodiment, the case where the first tapered surface **52a** of the pipe expansion punch **50** has the taper angle  $\alpha$  (refer to FIG. 1B or the like) is described. However, as shown in FIGS. 4A and 4B, a pipe expansion punch **80** having the taper angle  $\alpha$  of  $0^\circ$  may be press-fitted into the hollow shell **1** to form the hollow shell **1** into the intermediate formed product **90**. In this case, it is possible to further prevent deformation of the thin section **1a** (a decrease in the thickness of the thin section **1a**), and it is possible to reliably prevent the occurrence of defects in the thin section **1a**.

In addition, as shown in FIGS. 5A and 5B, the hollow shell **1** may be expanded and formed using the pipe expansion punch **80** having a cutout part **85** at the tip and a stationary die **100** having a bottom wall section **101** and a side wall section **102**. In this case, since the cutout part **85** is provided, the pipe expansion punch **80** can be smoothly pushed into the hollow shell **1**. Moreover, preferably, a gap between the first tapered surface **52a** and the side wall section **102** of the stationary die **100** is set to be 0.9 to 0.99 times the thickness of the hollow shell **1**. In this case, occurrence of deformation at the thin section **1a** can be more reliably prevented.

In addition, in the present embodiment, the case where the hollow shell **1** having the thin section **1a** provided at one location is expanded and formed is shown. However, as shown in FIG. 6A, a hollow shell **5** having the thin sections **1a** provided at two locations may be expanded and formed. In this case, similarly to the present embodiment, it is possible to prevent the occurrence of defects in the thin section **1a** using a pipe expansion punch **110** shown in FIGS. 6A and 6B.

Moreover, as shown in FIG. 7A, a hollow shell **7** having the thin sections **1a** provided at three locations may be expanded and formed. In this case, similarly to the present embodiment, it is possible to prevent the occurrence of defects in the thin section **1a** using the pipe expansion punch **120** shown in FIGS. 7A and 7B.

## Second Embodiment

Next, a second embodiment of the present invention will be described.

In the above-described first embodiment, the case where the flaring-processed metal pipe **20** is manufactured from the hollow shell **1** using the pipe expansion punch **50** and the forming punch **60** is described. Meanwhile, in the present embodiment, a flaring-processed metal pipe **220** shown in FIG. 8C is manufactured from the hollow shell **1** using a pipe expansion punch **250** shown in FIG. 8A.

As shown in FIG. 8A, the pipe expansion punch **250** has a cylindrical section **251** and a tapered section **252**. The pipe expansion punch **250** is different from the pipe expansion punch **50** of the first embodiment in that the cylindrical section **251** and the tapered section **252** are formed along the same central axis **CL5**.

Similarly to the case of the first embodiment, in the method of manufacturing the flaring-processed metal pipe **220** according to the present embodiment, the pipe expansion punch **250** is press-fitted into the hollow shell **1**. FIG. 8B is a view showing a state in which the pipe expansion

punch **250** is press-fitted to a predetermined position in the hollow shell **1**. In the state shown in FIG. 8B, the thick section **1b** of the hollow shell **1** abuts the cylindrical section **251** of the pipe expansion punch **250**, and the thin section **1a** of the hollow shell **1** abuts the tapered section **252** of the pipe expansion punch **250**.

FIG. 8C is a view showing a state in which the pipe expansion punch **250** is further press-fitted into the hollow shell **1** from the state shown in FIG. 8B. As shown in FIG. 8C, the flaring-processed metal pipe **220** can be obtained by press-fitting the pipe expansion punch **250** into the hollow shell **1** until the thin section **1a** abuts the cylindrical section **251** of the pipe expansion punch **250**.

In the present embodiment, since the taper angle  $\beta$  of the second tapered surface **52b** which abuts the thick section **1b** is larger than the angle  $\alpha$  of the first tapered surface **52a** which abuts the thin section **1a**, the thick section **1b** is preferentially subjected to tensile processing. That is, similarly to the case of the first embodiment, it is possible to prevent occurrence of forming defects in the thin section **1a** by allowing the thickness reduction rate of the thin section **1a** to be smaller than the thickness reduction rate of the thick section **1b**.

## EXAMPLE

Next, examples conducted for confirming effects of the present invention will be described.

According to the manufacturing method of the first embodiment, three kinds of flaring-processed metal pipes having different diameters of the pipe expanded sections were manufactured. In addition, for comparison, a flaring-processed metal pipe was manufactured according to a related art in which a flaring-processed metal pipe was manufactured using only a forming punch. In the flaring-processed metal pipes, the forming defects were evaluated by visually checking the presence or absence of breakage.

### Example 1

#### (1) Hollow Shell

As the hollow shell **1**, a seamless steel pipe having 73 mm in the outer diameter and 6 mm in the average thickness was used. The thickness of the thin section **1a** of the hollow shell **1** was 5.6 mm, and the thickness of the thick section **1b** of the hollow shell **1** was 6.4 mm.

#### (2) Punch

The pipe expansion punch **50** and the forming punch **60** were used.

In the pipe expansion punch **50**, the taper angle  $\alpha$  was  $4.5^\circ$ , the taper angle  $\beta$  was  $24.6^\circ$ , and the diameter of the cylindrical section **51** was 81.2 mm. In the forming punch **60**, the taper angle  $\gamma$  was  $15^\circ$ , and the diameter of the cylindrical section **61** was 81.2 mm.

#### (3) Stationary Die

In the stationary die **70**, the inner diameter  $D$  (refer to FIG. 3) of the side wall sections **72** was 93.2 mm.

#### (4) Manufacturing Process

The intermediate formed product **10** was manufactured by pushing the pipe expansion punch **50** into the hollow shell **1** to expand the hollow shell **1**. At this time, the intermediate formed product **10** was manufactured such that  $L1$  shown in FIG. 2 was 0.17 times  $L2$ .

Thereafter, the intermediate formed product **10** was disposed on the stationary die **70** and the forming punch **60** was pushed into the intermediate formed product **10** to manufacture the flaring-processed metal pipe **20**.

## 11

## (5) Evaluation of Forming Defects

Forming defects such as cracks did not occur in the intermediate formed product **10** and the flaring-processed metal pipe **20**. In addition, the pipe expansion rate of the flaring-processed metal pipe **20** was 30%.

## Example 2

## (1) Hollow Shell

As the hollow shell **1**, an electric resistance welded steel pipe having 90.0 mm in the outer diameter and 2.8 mm in the average thickness was used. In the electric resistance welded steel pipe, the tensile strength TS was 80 kgf/mm<sup>2</sup> (785 MPa), and the hardness distribution in the circumferential direction was the distribution shown in FIG. 9.

## (2) Punch

The pipe expansion punch **50** and the forming punch **60** were used.

In pipe expansion punch **50**, the taper angle  $\alpha$  was 4.5°, the taper angle  $\beta$  was 24.6°, and the diameter of the cylindrical section **51** was 112.4 mm.

In the forming punch **60**, the taper angle  $\gamma$  was 15°, and the diameter of the cylindrical section **61** was 112.4 mm.

## (3) Stationary Die

In the stationary die **70**, the inner diameter D (refer to FIG. 3) of the side wall sections **72** was 117 mm.

## (4) Manufacturing Process

The intermediate formed product **10** was manufactured by pushing the pipe expansion punch **50** into the hollow shell **1** to expand the hollow shell **1**. At this time, the intermediate formed product **10** was manufactured such that L1 shown in FIG. 2 was 0.17 times L2.

Thereafter, the intermediate formed product **10** was disposed on the stationary die **70** and the forming punch **60** was pushed into the intermediate formed product **10** to manufacture the flaring-processed metal pipe **20**.

## (5) Evaluation of Forming Defects

Forming defects such as cracks did not occur in the intermediate formed product **10** and the flaring-processed metal pipe **20**. In addition, the pipe expansion rate of the flaring-processed metal pipe **20** was 30%.

## Example 3

## (1) Hollow Shell

As a hollow shell **1**, the same electric resistance welded steel pipe as that of Example 2 was used.

## (2) Punch

The pipe expansion punch **50** and the forming punch **60** were used.

In the pipe expansion punch **50**, the taper angle  $\alpha$  was 7.5°, the taper angle  $\beta$  was 21.9°, and the diameter of the cylindrical section **51** was 129.4 mm.

In the forming punch **60**, the taper angle  $\gamma$  was 15°, and the diameter of the cylindrical section **61** was 129.4 mm.

## (3) Stationary Die

In the stationary die **70**, the inner diameter D (refer to FIG. 3) of the side wall sections **72** was 135 mm.

## (4) Manufacturing Process

Similarly to Examples 1 and 2, the intermediate formed product **10** was manufactured. In addition, in the present example, the intermediate formed product **10** was manufactured such that L1 shown in FIG. 2 was 0.33 times L2.

## (5) Evaluation of Forming Defects

Forming defects such as cracks did not occur in the intermediate formed product **10** and the flaring-processed

## 12

metal pipe **20**. In addition, the pipe expansion rate of the flaring-processed metal pipe **20** was 50%.

## Reference Example 1

5

## (1) Hollow Shell

The same electric resistance welded steel pipe as that of Example 2 was used.

## (2) Punch

Unlike Examples 1 to 3, the pipe expansion punch **50** was not used, and only the forming punch **60** was used

## (3) Stationary Die

The same stationary die **70** as that of Example 2 was used.

## (4) Manufacturing Process

The hollow shell **1** was disposed in the stationary die **70**, the forming punch **60** was pushed into the hollow shell **1** to expand the hollow shell, and the flaring-processed metal pipe was manufactured.

## (5) Evaluation of Forming Defects

The pipe expansion rate of the flaring-processed metal pipe was 30%, and the forming defects such as cracks did not occur in the flaring-processed metal pipe. In addition, in the present reference example, since the pipe expansion rate was as low as 30%, it was considered that forming defects did not occur even when the pipe expansion punch **50** was not used.

## Comparative Example 1

30

## (1) Hollow Shell

The same electric resistance welded steel pipe as that of Example 2 was used.

## (2) Punch

Unlike the above-described Examples 1 to 3, the pipe expansion punch **50** was not used, and only the forming punch **60** was used (that is, the same as Reference Example 1).

## (3) Die

The same stationary die **70** as that of Example 2 was used.

## (4) Manufacturing Process

The hollow shell **1** was disposed in the stationary die **70**, the forming punch **60** was pushed into the hollow shell **1** to expand the hollow shell, and the flaring-processed metal pipe was manufactured.

## (5) Evaluation of Forming Defects

The pipe expansion rate of the flaring-processed metal pipe was 50%, and cracks occurred in the flaring-processed metal pipe.

According to Examples 1 to 3, even when the low deformation resistance section having a small deformation resistance in the circumferential direction and a high deformation resistance section having a deformation resistance which is greater than that of the low deformation resistance section existed in the hollow shell **1**, it was possible to prevent forming defects such as cracks without applying a burden onto the low deformation resistance section.

Particularly, according to the comparison between Example 3 and Comparative Example 1, with respect to a product having a high pipe expansion rate in which cracks were generated in the related art, it was configured that the product could be manufactured without occurrence of cracks.

Hereinbefore, the embodiments of the present invention are described, the embodiments are suggested by way of example, and the scope of the present invention is not limited to the embodiments. The embodiments can be embodied in other various forms, and various omissions,

## 13

replacements, and modifications can be performed within the scope which does not depart from the gist of the present invention. The embodiments and the modifications are included in the scope and gist of the invention, and similarly, are also included in the inventions described in claims and the equivalent scopes.

For example, in the first embodiment, the case where the hollow shell **1** is formed into the intermediate formed product **10** using a pipe expansion punch **50** is described. However, the hollow shell **1** may be formed stepwise (at a plurality of times) using a plurality of pipe expansion punches having different outer diameters.

In addition, for example, in the first embodiment, the case where the intermediate formed product **10** is formed into the flaring-processed metal pipe **20** using the forming punch **60** is described. However, the intermediate formed product **10** obtained by the pipe expansion punch **50** without using the forming punch **60** may be the flaring-processed metal pipe. In this case, it is possible to obtain an eccentric flaring-processed metal pipe.

## INDUSTRIAL APPLICABILITY

According to the present invention, a method of manufacturing a flaring-processed metal pipe can be provided, in which it is possible to prevent occurrence of forming defects such as breakage when a flaring-processed metal pipe is manufactured from a hollow shell including a portion having a relatively small deformation resistance.

## BRIEF DESCRIPTION OF THE REFERENCE NUMERALS

**1:** hollow shell

**1a:** thin section (low deformation resistance section)

**1b:** thick section (high deformation resistance section)

**10:** intermediate formed product

**20:** flaring-processed metal pipe

**50:** pipe expansion punch

**60:** forming punch

**70:** stationary die

The invention claimed is:

1. A method of manufacturing a flaring-processed metal pipe having a pipe expanded section from a hollow shell including a plurality of portions having different deformation resistances when viewed in a circumferential direction, the method comprising:

among the plurality of portions spaced in the circumferential direction, specifying one of the plurality of portions as a low deformation resistance section having a first deformation resistance, and another of the plurality of portions as a high deformation resistance section having a second deformation resistance, the second deformation resistance being greater than the first deformation resistance; and

press-fitting a pipe expansion punch into the hollow shell and expanding the hollow shell, so that a thickness reduction rate of the low deformation resistance section is smaller than a thickness reduction rate of the high deformation resistance section.

2. The method of manufacturing a flaring-processed metal pipe according to claim 1, wherein the pipe expansion punch includes a first abutment surface which abuts the low deformation resistance section of the hollow shell, and a second abutment surface which abuts the high deformation resistance section of the hollow shell, and an inclination angle of the first abutment surface with respect to the central

## 14

axis of the pipe expansion punch is smaller than an inclination angle of the second abutment surface with respect to the central axis, and

wherein in the press-fitting and the expanding, the pipe expansion punch is press-fitted into the hollow shell while the first abutment surface of the pipe expansion punch abuts the low deformation resistance section of the hollow shell and the second abutment surface of the pipe expansion punch abuts the high deformation resistance section of the hollow shell.

3. The method of manufacturing a flaring-processed metal pipe according to claim 2, wherein the inclination angle of the first abutment surface of the pipe expansion punch is 0°.

4. The method of manufacturing a flaring-processed metal pipe according to claim 3, wherein the press-fitting and the expanding include:

press-fitting the pipe expansion punch into the hollow shell to obtain an intermediate formed product from the hollow shell; and

press-fitting a forming punch having a shape which coincides with an inner surface of the pipe expanded section of the flaring-processed metal pipe into the intermediate formed product.

5. The method of manufacturing a flaring-processed metal pipe according to claim 4, wherein the hollow shell is an electric resistance welded steel pipe or a seamless steel pipe.

6. The method of manufacturing a flaring-processed metal pipe according to claim 4, wherein in the press-fitting of the pipe expansion punch, the pipe expansion punch is press-fitted into the hollow shell such that a diameter expansion amount of the low deformation resistance section of the hollow shell is less than 0.5 times a diameter expansion amount of the high deformation resistance section of the hollow shell.

7. The method of manufacturing a flaring-processed metal pipe according to claim 6, wherein the hollow shell is an electric resistance welded steel pipe or a seamless steel pipe.

8. The method of manufacturing a flaring-processed metal pipe according to claim 3, wherein the hollow shell is an electric resistance welded steel pipe or a seamless steel pipe.

9. The method of manufacturing a flaring-processed metal pipe according to claim 2, wherein the press-fitting and the expanding include:

press-fitting the pipe expansion punch into the hollow shell to obtain an intermediate formed product from the hollow shell; and

press-fitting a forming punch having a shape which coincides with an inner surface of the pipe expanded section of the flaring-processed metal pipe into the intermediate formed product.

10. The method of manufacturing a flaring-processed metal pipe according to claim 9, wherein the hollow shell is an electric resistance welded steel pipe or a seamless steel pipe.

11. The method of manufacturing a flaring-processed metal pipe according to claim 9, wherein in the press-fitting of the pipe expansion punch, the pipe expansion punch is press-fitted into the hollow shell such that a diameter expansion amount of the low deformation resistance section of the hollow shell is less than 0.5 times a diameter expansion amount of the high deformation resistance section of the hollow shell.

12. The method of manufacturing a flaring-processed metal pipe according to claim 11, wherein the hollow shell is an electric resistance welded steel pipe or a seamless steel pipe.

**15**

13. The method of manufacturing a flaring-processed metal pipe according to claim 2, wherein the hollow shell is an electric resistance welded steel pipe or a seamless steel pipe.

14. The method of manufacturing a flaring-processed metal pipe according to claim 2, wherein the first abutment surface and the second abutment surface are sections of a conical surface.

15. The method of manufacturing a flaring-processed metal pipe according to claim 1, wherein the hollow shell is an electric resistance welded steel pipe or a seamless steel pipe.

16. The method of manufacturing a flaring-processed metal pipe according to claim 1, wherein the low deformation resistance section has a smaller thickness than the high deformation resistance section.

**16**

\* \* \* \* \*